# EUROPEAN PATENT SPECIFICATION

(11) **EP 1 811 054 B1**
(45) Date of publication and mention of the grant of the patent: **18.08.2010**
(21) Application number: 05759319.6
(22) Date of filing: 07.06.2005
(51) Int. Cl.: C22C 38/60, C21D 8/10

(54) **PIPE FOR PETROLEUM AND GAS PRODUCT PIPELINES AND METHOD FOR THE PRODUCTION THEREOF**
ROHR FÜR ERDÖL- UND GASPRODUKTPIPELINES UND HERSTELLUNGSVERFAHREN DAFÜR
CANALISATION POUR OLEODUCS ET GAZODUCS, ET PROCEDE DE FABRICATION ASSOCIE

(30) Priority: 07.06.2004 RU 2004117180
(43) Date of publication of application: 25.07.2007
(73) Proprietor: Kilkenny Industries S.A. (BVI), 9491 Ruggell (LI)
(72) Inventor: DUB, Vladimir Semyonovich, Moscow, 119285 (RU); MARKOV, Sergey Ivanovich, Moscow, 113534 (RU); LOBODA, Alexandr Sergeevich, Moscow, 107370 (RU); GOLOVIN, Sergey Vladimirovich, Moscow, 127322 (RU); BOLOTOV, Alexandr Semyonovich, Moskovskaya obl., 142117 (RU); DUB, Alexey Vladimirovich, Moscow, 121059 (RU); ROSCHIN, Maxim Borisovich, Moscow, 125047 (RU); GOSHKADERA, Sergey Vladimirovich, Moscow, 125368 (RU)
(74) Representative: Einsel, Martin
(86) International application number: PCT/RU2005/000314
(87) International publication number: WO 2005/121385

(56) References cited:
- EP-A- 1 705 260
- WO-A-99/05328
- DE-C1- 19 838 673
- JP-A- 2001 152 248
- RU-C1- 2 180 691
- RU-C2- 2 221 875
- US-A- 5 876 521
- US-B2- 6 565 682

## Description

### FIELD OF INVENTION

This invention relates to metallurgy, referring specifically to welded pipe production for oil pipelines, natural gas pipelines, product pipelines and other similar designs (tanks, pressure vessels) which can be safely operated in adverse geological and climatic conditions, and in aggressive corrosive liquids.

### STATE OF ART

The pipe and its method of manufacture is known (Patent of the Russian Federation No. 2180691, C 21 D9/08, publication of 10.11.1999). It includes steelmaking, ladle processing, steel teeming, hot rolling (several rolling passages with predetermined deformation ratio), shape molding and welding. Steel is molten from first or clean melting stock, with the following component ratio (weight, %):

| | |
|---|---|
| Carbon | 0.03 - 0.11 |
| Manganese | 0.9 -1.8 |
| Silicium | 0.06 - 0.6 |
| Chrome | 0.005 - 0.30 |
| Nickel | 0.005 - 0.3 |
| Vanadium | 0.02-0.12 |
| Niobium | 0.03-0.1 |
| Titanium | 0.01-0.04 |
| Aluminium | 0.01-0.055 |
| Calcium | 0.001-0.005 |
| Sulphur | 0.0005-0.008 |
| Phosphorus | 0.0005-0.010 |
| Nitrogen | 0.001-0.012 |
| Copper | 0.005-0.25 |
| Stibium | 0.0001-0.005 |
| Stannum | 0.0001-0.007 |
| Arsenic | 0.0001-0.008 |
| Iron | remaining share |

At this ratio the content of carbon, nitrogen, copper, phosphorus, stibium, stannum and arsenic shall be as follows:$C + 10 ⁢ N < 0.14$$10 ⁢ P + C ⁢ u < 0.14$$2 ⁢ P + S ⁢ n + S ⁢ b + A ⁢ s < 0.035$

During hot rolling deformation ratio in each rolling passage shall be 1.25-2.5 times less than in the previous one, and will be done in the following temperature range: ${T}_{b ⁢ g ⁢ n} - {T}_{e ⁢ n ⁢ d} < 200 ,$
where T_{bgn} and T_{end} are values of temperature at the start of hot roll and at the finish, accordingly.

Since this manufacturing method of pipes from hot-rolled sheets lacks fast controlled cooling, it results in sharp limitations on the manufacture of high-strength pipes (class K60 and above), especially with sheet thickness in excess of 12 mm, because such important properties of pipes as impact strength in subzero temperatures, plasticity, weldability, crack resistance and resistance to corrosion decrease. This is due to the fact that fast cooling, which is not envisaged in the invention, can be compensated by temperature reduction in the end of hot rolling down to 700°C -750°C and an increase of carbon and manganese content, in order to provide required strength properties at the level of 60 kg/mm² and more. Both methods provide the strength required, but they result in worse properties pertaining to as impact strength, weldability and resistance to corrosion.

### ESSENSE OF INVENTION

The purpose of this invention is to provide combination of the required strength properties (breaking strength above 620 kg/mm²) and high plasticity, ductility, crack resistance and resistance to corrosion in pipes and other products made from steel sheets up to 50 mm thick.

The object of the invention is solved by a method comprising the steps as mentioned in claim 1.

A co-pending European patent application post-published under EP-A-1 705 260 of the same applicant discloses a steel composition which is intended for the production of pipe lines and includes a steel composition including among others molybdenum. However, said document is not discussing a method for the production of pipe for oil products, natural gas products, product pipe lines.

Therefore, the following is an explanation of a respective method for solving the object of the invention.

Technically, the required result is obtained due to the fact that pipes for oil and gas pipelines are made of steel molten from first or clean melting stock with the following component ratio (weight, %):

| | |
|---|---|
| Carbon | 0.02 - 0.11 |
| Manganese | 0.10 -1.8 |
| Silicium | 0.06 - 0.6 |
| Chrome | 0.005 - 0.30 |
| Nickel | 0.005 - 1.0 |
| Vanadium | 0.01-0.12 |
| Niobium | 0.02-0.1 |
| Titanium | 0.01-0.04 |
| Aluminium | 0.01-0.05 |
| Calcium | 0.0005-0.008 |
| Sulphur | 0.0005-0.008 |
| Phosphorus | 0.001-0.012 |
| Nitrogen | 0.001-0.012 |
| Copper | 0.005-0.25 |
| Stibium | 0.0001-0.005 |
| Stannum | 0.0001-0.007 |
| Arsenic | 0.0001-0.008 |
| Molybdenum | 0.0001-0.5 |
| Iron | remaining share, |

this being the case, total content of nickel and manganese is related to molybdenum and phosphorus content (weight. %) according to the following equation: $\frac{Ni + Mn}{1 + Mo} ⋅ P < 0.03$

Also, the required result is obtained due to the fact that the method for production of the above pipe includes steelmaking with the above content ratio, ladle processing, hot rolling, shape molding and welding of pipes. This being the case, hot rolling is performed in reversing mill or continuous mill with subsequent fast controlled cooling, its rate being determined by the following equation: $\frac{\left({T}_{hot}-{T}_{cold}\right)}{Ls} ⁢ {V}_{s} , °C / sec$

Rate value in the process shall be according to the following: $\frac{\left({T}_{hot}-{T}_{cold}\right)}{Ls} ⁢ {V}_{s} > 4 ,$
where
Tₕₒₜ is the temperature of steel sheet or steel band in the end of rolling, its value being within 750°C -850°C range;
T_{cold} is the temperature of steel sheet or steel band in the end of fast controlled cooling, its value being within 500°C -700°C range;
Vₛ is the steel sheet or steel band speed in the sprinkler or laminar flow, m/sec;
Lₛ is the length of sprinkler or laminar unit (can be changed in the 10-100 m range).

These inventions can simultaneously provide the required strength properties (breaking strength increases) of steel sheets up to 50 mm thick, their ductility in subzero temperatures, weldability, crack resistance and resistance to corrosion, provided the above component ratio is observed.

### EXAMPLES OF REALIZATION OF INVENTION

Table 1 shows the chemical composition of steel in two pipes, one made in accordance with the composition offered and the other one - of a different composition. The compositions were selected in such a way so as to estimate molybdenum and nickel contribution to steel sheet strength in different cooling conditions after rolling. Melting process was performed in a vacuum induction furnace. Furnace charge consisted of armco iron and, depending on variant of composition, of nickel, ferromolybdenum, copper and other charge materials. When the required underpressure in the furnace was achieved charge meltdown was started. After complete meltdown and metal heating up to 1630°C -1650°C the charge was degasified and the required predetermined amounts of manganese, ferrovanadium and ferroniobium were added to the molten pool; then deoxidizing agents (ferrosilicium, aluminium and ferrotitanium) were added. As the temperature of liquid steel reached the required level (1560°C -1580°C) the airfree metal was run off directly from the smelting crucible to the casting mold.

On the whole, 12 trial heats have been performed in the vacuum induction furnace. Analysis of metal chemical composition has been performed for each heat. On the basis of its results three heats have been selected where the ratio between the total content of nickel and manganese and the concentration of molybdenum and phosphorus for heats 1,2 and 3 is 0.01, 0.0057 and 0.0064, respectively, i.e. less than 0.03.

The ingots selected and the molten steel of a given pipe were forged into 80-430 mm plates; then they were rolled in a reversing mill to become 50 and 20 mm thick. After that the plates were fast-cooled at a rate of 10 and 20 degrees per second and alternately cooled in the open air. The latter cooling procedure corresponds to hot-rolled sheet conditions while the first two - to controlled fast cooling. The resulting sheets were then shaped and welded into pipes.

Table 2 shows the properties of these heats in comparison with heats of a known composition. The obtained results demonstrate that the new steel of the above composition made in accordance with the offered rolling technology, which involves controlled cooling at a rate of 4°C per second, has the required combination of properties, such as high strength in 50-mm cross-sections and high tenacity, and therefore, good crack resistance and ductility in subzero temperatures. The 10 m/sec sheet passage speed in controlled cooling has been obtained in a wide-strip rolling mill. The sheet surface temperature at the end of rolling mill was 840°C; The sheet surface temperature at the end of controlled cooling procedure was 640°C; the length of laminary machine - 60 m; the steel strip movement speed in the laminar stream - 3 m/sec. The 20 m/sec sheet passage speed in controlled cooling has been obtained in a reversing mill. The sheet surface temperature at the end of rolling mill was 800°C; The sheet surface temperature at the end of controlled cooling procedure was 600°C; the length of quench sprinkler was 10 m, the steel strip movement speed in the sprinkler was 1 m/sec. The rate of steel sheet air cooling was approximately 2-3°C/sec. After cooling the sheet is shaped into pipe and its edges are welded.

| Table 1 | | | | |
|---|---|---|---|---|
| Component | Content (weight %) | | | |
| | Heat 1 | Heat 2 | Heat 3 | Heat of known steel |
| carbon | 0.02 | 0.04 | 0.09 | 0.06 |
| manganese | 1.5 | 1.0 | 0.3 | 1.4 |
| silicium | 0.1 | 0.18 | 0.25 | 0.25 |
| chrome | 0.05 | 0.28 | 0.2 | 0.15 |
| nickel | 0.5 | 0.1 | 0.9 | 0.1 |
| vanadium | 0.1 | 0.05 | 0.01 | 0.07 |
| niobium | 0.032 | 0.06 | 0.087 | 0.06 |
| titanium | 0.01 | 0.015 | 0.035 | 0.015 |
| aluminium | 0.012 | 0.021 | 0.028 | 0.024 |
| calcium | 0.0005 | 0.003 | 0.006 | 0.005 |
| sulphur | 0.0035 | 0.004 | 0.008 | 0.003 |
| phosphorus | 0.005 | 0.007 | 0.008 | 0.005 |
| nitrogen | 0.005 | 0.006 | 0.007 | 0.007 |
| copper | 0.23 | 0.1 | 0.01 | 0.15 |
| stibium | 0.0003 | 0.0009 | 0.004 | 0.005 |
| stannum | 0.0005 | 0.005 | 0.007 | 0.005 |
| arsenic | 0.0002 | 0.004 | 0.008 | 0.006 |

**Table 2**

| Steel properties | | | | | | | |
|---|---|---|---|---|---|---|---|
| Heat | Sheet thickness, mm | Breaking strength, N/mm² | | | Ductile-brittle transition point, °C | | |
| | | Cooling rate, °C | | | Cooling rate °C | | |
| | | 20 | 10 | Air | 20 | 10 | Air |
| 1 | 20/50 | 836/687 | 780/730 | 550/470 | -90/-80 | -80/-70 | -50/-40 |
| 2 | 20/50 | 807/712 | 750/650 | 540/460 | -90/-80 | -80/-70 | -50/-40 |
| 3 | 20/50 | 767/657 | 720/630 | 530/450 | -90/-80 | -80/-70 | -50/-40 |
| Heat of known steel | 20/50 | 621/528 | 500/410 | 420/340 | -80/-30 | -50/-20 | -20/-10 |

## Claims

1. Method for the production of pipe for oil products, natural gas products, product pipelines including steelmaking a steel having a composition with the following component ratio (weight %):
| | |
|---|---|
| Carbon | 0.02 - 0.11 |
| Manganese | 0.10 - 1.8 |
| Silicium | 0.06 - 0.6 |
| Chrome | 0.005 - 0.30 |
| Nickel | 0.005 - 1.0 |
| Vanadium | 0.01 - 0.12 |
| Nioblum | 0.02 - 0.1 |
| Titanium | 0.01 - 0.04 |
| Aluminium | 0.01 - 0.05 |
| Calcium | 0.0005 - 0.008 |
| Sulphur | 0.0005 - 0.008 |
| Phosphorous | 0.001 - 0.012 |
| Nitrogen | 0.001 - 0.012 |
| Copper | 0.005 - 0.25 |
| Stibium | 0.0001 - 0.005 |
| Stannum | 0.0001 - 0.007 |
| Arsenic | 0.0001 - 0.008 |
| Molybdenum | |
| Iron | remaining share, |
whereby the total content of nickel and manganese is related to molybdenum and phosphorus content (weight %) according to the following equation: $\frac{Ni + Mn}{1 + Mo} ⋅ P < 0.03 ,$
ladle processing, steel teeming, hot rolling, shape molding and welding,
wherein hot rolling is realized in reversing mill or continuous mill with subsequent fast controlled cooling, its rate being determined by the following equation: $\frac{\left({T}_{hot}-{T}_{cold}\right)}{Ls} ⁢ {V}_{s} , °C / sec ,$
said rate value in the process shall be according to the following: $\frac{\left({T}_{hot}-{T}_{cold}\right)}{Ls} ⁢ {V}_{s} > 4 ,$
where
Tₕₐₜ is the temperature of steel sheet or steel band in the end of rolling, its value being within 750 ºC -850°C range;
T_{cold} is the temperature of steel sheet or steel band in the end of fast controlled cooling, its value being within 500 °C -700 ºC range;
Vₛ is the steel sheet or steel band speed in the sprinkler or laminar flow, m/sec;
Lₛ is the length of sprinkler or laminar unit which can differ between 10-100 meters.

## Patentansprüche

1. Verfahren zur Herstellung von Rohren für Ölprodukte, Erdgasprodukte, Produktpipelines einschließlich des Herstellens von Stahl für einen Stahl mit einer Zusammensetzung mit den folgenden Verhältnissen der Komponenten (in Gewichtsprozent):
| | |
|---|---|
| Kohlenstoff | 0,02-0,11 |
| Mangan | 0,10-1,8 |
| Silizium | 0,06-0,6 |
| Chrom | 0,005-0,30 |
| Nickel | 0,005-1,0 |
| Vanadium | 0,01-0,12 |
| Niob | 0,02-0,1 |
| Titan | 0,01-0,04 |
| Aluminium | 0,01-0,05 |
| Kalzium | 0,0005-0,008 |
| Schwefel | 0,0005-0,008 |
| Phospor | 0,001-0,012 |
| Stickstoff | 0,001-0,012 |
| Kupfer | 0,005-0,25 |
| Antimon | 0,0001-0,005 |
| Zinn | 0,0001-0,007 |
| Arsen | 0,0001-0,008 |
| Molybdän | 0,0001-0,5 |
| Eisen | restlicher Anteil, |
wobei der Gesamtgehalt an Nickel und Mangan sich in Bezug auf den Gehalt an Molybdän und Phosphor (in Gewichtsprozent) gemäß der folgenden Gleichung verhält: $\frac{Ni + Mn}{1 + Mo} ⋅ P < 0 , 03 ,$
Schmelzverarbeitung, Stahlgussvorgänge, Warmwalzen, Formgießen und Schweißen,
wobei das Warmwalzen mit einem Umkehrwalzwerk oder einem kontinuierlichen Walzwerk mit folgendem schnellen geregelten Abkühlen durchgeführt wird, wobei die Abkühlgeschwindigkeit durch die folgende Gleichung festgelegt wird: $\frac{\left({T}_{hot}-{T}_{cold}\right)}{Ls} ⁢ {V}_{s} °C / sec$
wobei dieser Geschwindigkeitswert in dem Verfahren gemäß dem folgenden sein soll: $\frac{\left({T}_{hot}-{T}_{cold}\right)}{Ls} ⁢ {V}_{s} > 4 ,$
wobei Tₕₒₜ die Temperatur des Bleches oder Stahlbandes am Ende des Walzvorgangs ist, wobei dieser Wert in dem Bereich zwischen 750 °C und 850 °C liegt;
T_{cold} die Temperatur des Bleches oder Stahlbandes am Ende des schnellen geregelten Abkühlens ist, wobei dieser Wert in dem Bereich zwischen 500 °C und 700 °C liegt;
Vₛ die Geschwindigkeit des Bleches oder Stahlbandes in der Sprinkler- oder einer laminaren Strömung in m/s ist;
Lₛ die Länge der Sprinkler- oder Laminareinheit ist, welche zwischen 10 und 100 m liegen kann.

## Revendications

1. Procédé de production d'une canalisation pour produits pétroliers, produits gazeux, pipelines pour lesdits produits, comprenant les étapes consistant à fabriquer un acier ayant une composition dans laquelle le rapport des composants (en % massique) est le suivait :
| | |
|---|---|
| Carbone | 0,02 à 0,11 |
| Manganèse | 0,10 à 1,8 |
| Silicium | 0,06 à 0,6 |
| Chrome | 0,005 à 0,30 |
| Nickel | 0,005 à 1,0 |
| Vanadium | 0,01 à 0,12 |
| Niobium | 0,02 à 0,1 |
| Titane | 0,01 à 0,04 |
| Aluminium | 0,01 à 0,05 |
| Calcium | 0,0005 à 0,008 |
| Soufre | 0,0005 à 0,008 |
| Phosphore | 0,001 à 0,012 |
| Azote | 0,001 à 0,012 |
| Cuivre | 0,005 à 0,25 |
| Antimoine | 0,0001 à 0,005 |
| Etain | 0,0001 à 0,007 |
| Arsenic | 0,0001 à 0,008 |
| Molybdène | 0,0001 à 0,5 |
| Fer | Reste, |
dans lequel la teneur totale en nickel et en manganèse est fonction de la teneur en molybdène et en phosphore (en % massique), conformément à l'équation suivante : $\frac{Ni + Mn}{1 + Mo} ⋅ P < 0 , 03$
traiter ledit acier en poche de coulée, couler ledit acier, laminer à chaud ledit acier, mouler ledit acier, et souder ledit acier,
dans lequel le laminage à chaud est effectué sur train de laminage réversible ou continu, suivi d'un refroidissement rapide commandé, sa vitesse étant déterminée selon l'équation suivante : $\frac{\left({T}_{hot}-{T}_{cold}\right)}{Ls} ⁢ {V}_{s} , °C / sec ,$
la valeur de ladite vitesse dans le procédé étant déterminée comme suait : $\frac{\left({T}_{hot}-{T}_{cold}\right)}{Ls} ⁢ {V}_{s} > 4 ,$
où,
Tₕₒₜ est la température de la tôle ou de la bande d'acier à la fin du laminage, sa valeur allant de 750 °C à 850 °C ;
T_{cold} est la température de la tôle ou de la bande d'acier à la fin du refroidissement rapide commandé, sa valeur allant de 500 °C à 700 °C ;
Vₛ est la vitesse de passage de la tôle ou de la bande d'acier dans la machine à laminer, exprimée en m/sec ;
Lₛ est la longueur de la machine à laminer qui peut aller de 10 à 100 mètres.
